

Patented Sept. 4, 1945

2,384,006

# UNITED STATES PATENT OFFICE

2,384,006

## SCOURING AND POLISHING POWDER

Joseph M. Bleakney, Manhasset, N. Y.

No Drawing. Application March 18, 1943,  
Serial No. 479,595

6 Claims. (Cl. 252—129)

This invention relates to a cleaning composition which may be used for both scouring and polishing aluminum, porcelain, silver and many other materials.

Present day cleaning compositions may be divided roughly into scouring powders and polishing powders. In the former, the active cleaning agent is a pulverized material, such for example, as volcanic ash, having relatively large, hard particles which cut through dirt, grease, etc., when rubbed over the surface to be cleaned. Such powders remove the undesired substance and so clean the surfaces over which they are applied. But, at the same time, their gritty particles produce a multitude of scratches visible to the naked eye. On some surfaces this may not be particularly objectionable, but on others, especially relatively soft materials, such as silver, these scratches would be extremely objectionable.

Polishing powders comprise a very finely pulverized abrasive material which removes tarnish, stains, etc., without producing scratches visible to the naked eye. In such powders, the particles are so small that they will not cut through grease, scum, etc., and consequently these powders are not effective for scouring purposes.

Also, polishing powders when dry, have a tendency to pack together and therefore are not adaptable for use in containers with sifter openings. Furthermore, a dry powder produces an objectionable dust when shaken from the container. Accordingly, such powders are usually sold in liquid or paste carriers. Such arrangements increase the expense of the cleaning material not only by the cost of the carrying medium but they also require expensive air-tight containers to prevent deterioration of the liquid or paste.

The present cleaning composition not only scours and polishes in a single operation but it also has all the advantages of a dry powder which may be readily dispensed through a sifter opening without producing objectionable dust.

It has been found that when finely divided abrasive polishing powder is firmly attached to larger particles of a relatively soft material, the resulting composition may be used for both scouring and polishing purposes. The particles in this composition are sufficiently large to scour dirt, grease and other substances, over which ordinary polishing powder would smudge. At the same time, these particles, being of relatively soft material, are not sufficiently hard to produce scratches on the surfaces over which they are rubbed.

The relatively soft material, the particles of which may be considered as constituting the aggregate in the resulting mixture, may be any suitable substance which is not hard or gritty enough to scratch the surface being cleaned. Its particle size is not critical. A preferred substance is sawdust, obtained from either hard or soft wood. But ground cork or cornmeal, and many other materials, can be used.

10 The abrasive, or polishing powder is preferably finely ground diatomaceous earth but other polishing materials may be substituted according to the character of the surfaces to be cleaned. It is held on the aggregate by varnish, natural or artificial resin lacquers, animal or vegetable glues, or other suitable binders, being applied while the binder is still tacky.

15 A small percentage of either a so-called pure soap, or a "built" soap, i. e., one which comprising pure soap and an alkali, is added as a lubricant and water softener and for rinsing the surface. It has been found that approximately 5% of such soap powder is satisfactory.

20 It will be understood that the proportions of each of these ingredients may be varied over a wide range. By way of example, a preferred composition comprises, by volume:

|                    | Per cent |
|--------------------|----------|
| Sawdust            | 45       |
| Diatomaceous earth | 45       |
| Binder             | 5        |
| Powdered soap      | 5        |

25 Such a composition may be prepared as follows, using either hand or mechanical mixing apparatus:

30 The sawdust is mixed with the binder so that the latter is more or less evenly spread over the particles of sawdust. After the binder has partly dried, but while it is still tacky, the polishing powder is added and the mixture stirred, or tumbled, until this powder is thoroughly distributed over the sawdust particles. It is usually desirable to continue this mixing until the binder is dry, thus insuring greater and more uniform distribution of the polishing powder. When the mixture is thoroughly dry, the soap powder is added.

35 The resulting dry composition is used in the usual manner, i. e., applied to a damp cloth and rubbed over the surface to be cleaned.

40 What is claimed is:

45 1. A scouring and polishing powder comprising sawdust, the particles of which are coated with a dried binder, finely ground diatomaceous

earth securely imbedded in said binder and a dry soap powder.

2. A scouring and polishing powder comprising sawdust, the particles of which are coated with a dried binder, finely ground diatomaceous earth securely imbedded in said binder and a powdered soap.

3. A scouring and polishing powder comprising cellulosic material having relatively soft particles coated with a dried binder, finely ground diatomaceous earth securely imbedded in said binder and powdered soap.

4. A cleaning composition comprising cellulosic material having relatively soft particles coated with a dried binder, finely divided mineral abrasive polishing powder securely imbedded in said

binder and a dry soap powder mixed with said coated particles.

5. A cleaning composition comprising cellulosic material having relatively soft particles coated with a dried binder, finely divided mineral abrasive polishing powder securely imbedded in said binder and a powdered soap mixed with said coated particles.

10 6. A combined scouring and polishing powder comprising by volume about forty-five percent sawdust, forty-five percent diatomaceous earth, five per cent dried binder and five percent soap powder, said binder acting to hold the particles of said diatomaceous earth securely to said sawdust.

15 JOSEPH M. BLEAKNEY.